# EUROPEAN PATENT SPECIFICATION

(11) **EP 0 617 324 B1**
(45) Date of publication and mention of the grant of the patent: **14.05.1997**
(21) Application number: 94200769.1
(22) Date of filing: 24.03.1994
(51) Int. Cl.: G03C 7/392, G03C 7/413

(54) **Use of pyrazolidinone compounds to reduce granularity of photographic silver halide materials**
Verwendung von Pyrazolidinon-Verbindungen zur Verringerung der Granularität von photographischen Silberhalogenid-Materialien
Utilisation de composés pyrazolidinone pour réduire la granularité de matériaux photographiques à l'halogénure d'argent

(30) Priority: 26.03.1993 GB 9306355
(43) Date of publication of application: 28.09.1994
(73) Proprietor: KODAK LIMITED, Harrow, Middlesex HA1 4TY (GB)
(72) Inventor: Twist, Peter Jeffery, c/o Kodak Limited, Harrow, Middlesex HA1 4TY (GB)
(74) Representative: Nunney, Ronald Frederick Adolphe

(56) References cited:
- EP-A- 0 347 848
- EP-A- 0 347 849
- WO-A-92/10789

## Description

This invention relates to the use of pyrazolidinone compounds to reduce granularity of photographic silver halide materials and in particular colour negative materials.

There is a constant desire to improve the quality of photographic colour negative materials, particularly colour negative films, so as to obtain improved properties in the images formed after exposure and processing. These improvements are desirable but not at the expense of losing some other desirable property.

One such property is granularity or the perceived "graininess" of the dye image.

US patent 4 859 578 describes a photographic colour negative recording material which contains (1) an image dye-forming coupler, (2) a DIR compound, (3) a compound which releases a water-soluble mercaptan on silver halide development said to be invovled in selective development acceleration and (4) a compound which releases an electron transfer agent (ETA) on silver halide development. (Incidentally such materials very often contain developer inhibitor-releasing compounds (usually couplers) to improve properties such as sharpness in the image areas in the vicinity of its release). The material is said to have improved granularity without sacrificing other desirable properties. The present invention does not use incorporated compounds (3) or (4) which, of course, only act in the vicinity of their release.

US patent 4 526 863 describes a photographic colour negative recording material having a relatively light-insensitive silver halide, zinc oxide or titanium oxide layer positioned between two photosensitive silver halide layers which contains a compound which releases a fogging agent in the vicinity of silver halide development.

In contrast to the above two pieces of prior art, it is not essential to use incorporated fogging agent- or ETA-releasing compounds which only act in the vicinity of silver halide development in the present invention.

According to the present invention there is provided an invention comprising the use of a pyrazolidinone compound of the formula: or or a precursor thereof which releases the pyrazolidinone compound on treatment with an alkaline processing solution, to reduce the granularity of an imagewise exposed and processed photographic silver halide colour negative material comprising a support bearing at least one photosensitive silver halide emulsion layer having associated therewith a dye image-forming coupler and containing the pyrazolidinone compound in such amount that the granularity is reduced without any substantial change in dye density at the same level of exposure.

The invention provides a processed colour negative material having improved granularity without loss or gain of density for a given exposure. It is believed that mechanism by which the invention achieves its results is through an increase in silver development and the number of silver centres but with a lowering of dye yield per unit silver. This is especially true of the Dₘᵢₙ and fog regions.

The pyrazolidinones employed herein (which are electron transfer agents) are those which, at the correct level, can increase silver development, reduce dye yield such that the dye density is about the same as in the control case and reduce the gamma-normalised granularity.

The pyrazolidinones may be present in the colour negative material in an amount of from 0.01 to 5.0 g/m², preferably 0.05 to 1.0 g/m² and especially 0.2 to 0.8 g/m². They may be located in an emulsion layer or another layer of the material. Preferably they are located in or adjacent the silver halide emulsion layer nearest the support.

Preferably the incorporated material is a pyrazolidinone precursor which remains inactive until the material is treated with an alkaline processing solution. Such a precursor may beta compound of one of the formulae: or wherein R¹ and R² are alkyl or aryl groups that may be substituted. It is preferred that R¹ and R² are ballast groups of such a size and configuration to render the compound non wandering in photographic layers.

The pyrazolidinone may also be present in the colour developer in addition to the colour negative material. The amount of the pyrazolidone of formula (I) or (II) employed in the colour developer may range from 0.05 to 5.0 g/l, preferably from 0.1 to 1.0 g/l and particularly from 0.2 to 0.5 g/l As will be illustrated below in the Examples, the optimum amount can be determined by experiment.

The other electron transfer agents used as comparison examples in the Examples below illustrate different balances between silver development and dye yield. Those in Examples 2 and 3 cause a small increase in silver development but most of this is translated into dye resulting in an overall increase in density in the Dₘᵢₙ and toe region. This result is similar to over-development and gives an increase in granularity.

The electron transfer agent in Example 5 is one which causes a small increase in silver development but with a much reduced dye yield resulting in an overall reduction in dye density throughout the entire sensitometric curve. This causes a reduction in raw granularity but is accompanied by a loss of sensitometric response typical of other compounds which act as "toe-cutters".

The colour development step is preferably followed by the conventional bleach, fix (or bleach-fix) and wash and/or stabilise steps. A typical process is the C41 process described in British Journal of Photography (1988) pages 196-98. The exact composition, the temperature and the time of processing can be established by experiment.

The photographic material to be processed may be any of those described in Research Disclosure Item 308119, December 1989 published by Kenneth Mason Publications, Emsworth, Hants, United Kingdom.

The following Examples are included for a better understanding of the invention. They are model experiments in which the pyrazolidinone is located entirely in the colour developer but it is believed that the results obtained with the single layer coatings employed would be very similar if the pyrazolidinone were contained in the coated element.

### EXAMPLE 1 (Invention)

A single layer colour negative film (strip a) containing 1.0g/m² of silver in the form of a bromoiodide
T-Grain emulsion and 0.6g/sq.metre of a cyan coupler of the formula: was exposed to a test step wedge and processed by the following process what 38 °C:

| | |
|---|---|
| 1. Colour developer | 3.25 mins |
| 2. Bleach | 4.50 mins |
| 3. Wash | 1.00 mins |
| 4. Fix | 4.35 mins |
| 5. Stabilise | 1.00 mins |

### Colour developer

| | |
|---|---|
| DTPA | 6.5 ml |
| Sodium sulphite (anhy) | 4.25 g |
| Potassium iodide | 1.2 mg |
| Sodium bromide | 1.3 g |
| Hydroxylamine sulphate | 2.0 g |
| 4-(N-ethyl-N-2-hydroxyethyl)-2-methylphenylenediamine | 4.75 g |
| Water to | 1.0 litre |

pH = 10.0

DTPA is a 41% solution of the penta sodium salt of diethylenetriamine pentaacetic acid.

### Bleach

| | |
|---|---|
| Sodium iron (III) ethylenediamine-tetra-acetic acid | 100.0 g |
| Potassium bromide | 50.0 g |
| Acetic acid | 6.0 ml |
| Water to | 1.0 litre |

### Fixer

| | |
|---|---|
| Ammonium thiosulphate | 120.0 g |
| Sodium sulphite (anhy) | 20.0 g |
| Potassium metabisulphite | 20.0 g |
| Water to | 1.0 litre |

### Stabiliser

| | |
|---|---|
| Formaldehyde (36% soln) | 6.0 ml |
| Water to | 1.0 litre. |

Further strips of the same material were processed similarly except that the developer additionally contained 4'-methoxy-1-phenylpyrazolidin-3-one. In Figure 1 a comparison of 0, 0.15 (b) and 0.3g/l (c) of 4'-methoxy-1-phenylpyrazolidin-3-one (4MP) for a 2.5 minute development time shows a reduction in gamma normalised granularity with 4MP. This extends over most of the exposure scale. There is also a reduction of raw granularity particularly in the Dₘᵢₙ. It can be seen that the Dₘᵢₙ density increases with 4MP then comes down again. A photmicrographic examination shows that 4MP increases the number of developed silver centres in the Dₘᵢₙ and toe region of the sensitometric curve. In the Dₘᵢₙ region these extra silver centres are simply more fog grains but because the dye density is about the same (at 0.3g/l of 4MP) the granularity in the Dₘᵢₙ area is reduced. It appears that the granularity reduction carries on up the sensitometric curve but it is not certain that the mechanism is the same as in the Dₘᵢₙ and toe region. The results of a similar experiment but with a longer development time (5 minutes) is shown in Figure 2. Here the effects are essentially the same but more pronounced with a larger reduction in gamma-normalised and raw granularity. If the raw granularity in the Dₘᵢₙ is plotted against the level of ETA in the developer solution at differing development times then the plot in Figure 3 is obtained. In this plot it is clear that 4MP causes a reduction in granularity at all levels and prevents the increase in granularity at extended development times.

### Example 2 (Comparative)

This is a comparison example of a commercially used pyrazolidone, 4,4-dimethyl-1-phenyl-pyrazolidin-3-one. In Figure 4 the effect of adding the pyrazolidone to the developer of Example 1 at 0 (curve a), 0.15 (b) and 0.3g/l (c) is shown. There is an increase in dye density in the Dₘᵢₙ and toe of the curve and an increase in raw granularity. Gamma-normalised granularity is either unchanged or slightly higher depending on the exposure. This compound compares unfavourably with that used in Example 1.

### Example 3 (Comparative)

This is a comparison example with another pyrazolidone, 4,4-bis-hydroxymethyl-1-phenylpyrazolidin-3-one (BOP). In Figure 5 the effect of adding BOP to the developer of Example 1 at 0, 0.15 and 0.3g/l is shown. There is an increase in dye density in the Dₘᵢₙ and toe of the curve similar to that of Example 2. There is also an increase in raw granularity and in gamma-normalised granularity for most of the sensitometric curve. This compound compares unfavourably with that shown in Example 1.

Other pyrazolidones such as 1-phenylpyrazolidin-3-one and 4,4-hydroxymethyl-methyl pyrazolidin-3-one (MOP) behave similarly to those in Examples 2 and 3.

### Example 4 (Invention)

The procedure of Example 1 was repeated except that the pyrazolidone was replaced with 4'-ethoxy 1-phenylpyrazolidin-3-one. As can be seen from Figure 6, this lowers raw granularity and gamma-normalised granularity but to a lesser extent than 4'-methoxy-1-phenylpyrazolidin-3-one.

### Example 5 (Comparative)

This is a comparison example using the same method as above of a pyrazolidone that acts as a "toe cutter". 4-n-pentyl-1-phenylpyrazolidin-3-one lowers sensitometric response in terms of speed and Dₘᵢₙ even at low levels where Examples 1-4 show increases. This is shown in Figure 7. This compound lowers raw granularity by reducing the dye yield and, as shown by photomicrographic examination, leaving the number of developed silver grains approximately the same as in its absence.

## Claims

1. The use of a pyrazolidinone compound of the formula: or or a precursor thereof which releases the pyrazolidinone compound on treatment with an alkaline processing solution, to reduce the granularity of an imagewise exposed and processed photographic silver halide colour negative material comprising a support bearing at least one photosensitive silver halide emulsion layer having associated therewith a dye image-forming coupler and containing the pyrazolidinone compound in such amount that the granularity is reduced without any substantial change in dye density at the same level of exposure.

2. A use as claimed in claim 1 in which the precursor is a ballasted compound which releases the pyrazolidone when contacted with an alkaline colour developer solution.

3. A use as claimed in claim 2 in which the pyrazolidone precursor has one of the formulae: or wherein R¹ and R² are alkyl or aryl groups that may be substituted and wherein R¹ and R² are of such size and configuration to render the precursor non-wandering in photographic layers.

4. A use as claimed in any of claims 1-3 in which the colour negative material is a film containing from 0.01 to 5.0 g/m² of the pyrazolidinone.

5. A use as claimed in any of claims 1-3 in which the colour negative material is a film containing from 0.05 to 1.0 g/m² of the pyrazolidinone.

6. A use as claimed in any of claims 1-5 in which the colour developer solution used for processing the material also contains a pyrazolidinone of formula (I) or (II) as defined in claim 1.

7. A use as claimed in claim 6 in which the colour developer solution contains from 0.05 to 5.0 g/l of the pyrazolidinone.

8. A use as claimed in claim 6 in which the colour developer solution contains from 0.1 to 1.0 g/l of the pyrazolidinone.

9. A use as claimed in any of claims 1-8 in which the colour negative material is a multicolour photographic material comprising a support bearing a yellow dye image-forming unit comprised of at least one blue-sensitive silver halide emulsion layer having associated therewith at least one yellow dye-forming coupler, at least one magenta dye image-forming unit comprising at least one green-sensitive silver halide emulsion layer having associated therewith at least one magenta dye-forming coupler at least one cyan dye image-forming unit comprising at least one red-sensitive silver halide emulsion layer having associated therewith at least one cyan dye-forming coupler.

10. A use as claimed in any of claims 1-9 in which the pyrazolidinone is located in or adjacent the silver halide emulsion layer nearest the support.

## Patentansprüche

1. Verwendung einer Pyrazolidinon-Verbindung der Formel: oder oder einer Vorläuferverbindung hiervon, die die Pyrazolidinon-Verbindung bei Behandlung mit einer alkalischen Entwicklungslösung freisetzt, zur Verminderung der Körnigkeit eines bildweise exponierten und entwickelten farbphotographischen Silberhalogenid-Negativmaterials mit einem Träger, auf dem sich mindestens eine photosensitive Silberhalogenidemulsionsschicht befindet, der ein ein Farbbild bildender Kuppler zugeordnet ist, und das die Pyrazolidinon-Verbindung in einer solchen Menge enthält, daß die Körnigkeit vermindert wird ohne eine ins Gewicht fallende Veränderung der Farbstoffdichte bei dem gleichen Exponierungsgrad.

2. Verwendung nach Anspruch 1, bei der die Vorläuferverbindung eine Ballast aufweisende Verbindung ist, welche das Pyrazolidon bei Kontakt mit einer alkalischen Farbentwicklerlösung freisetzt.

3. Verwendung nach Anspruch 2, bei der die Pyrazolidon-Vorläuferverbindung eine der Formeln hat: oder worin R¹ und R² Alkyl- oder Arylgruppen darstellen, die substituiert sein können, und worin R¹ und R² von einer solchen Größe und Konfiguration sind, daß sie die Vorläuferverbindung in photographischen Schichten in eine nicht-wandernde Form überführen.

4. Verwendung nach einem der Ansprüche 1-3, bei der das Farb-Negativmaterial ein Film ist, der 0,01 bis 5,0 g/m² des Pyrazolidinons enthält.

5. Verwendung nach einem der Ansprüche 1-3, bei der das Farb-Negativmaterial ein Film ist, der 0,05 bis 1,0 g/m² des Pyrazolidinons enthält.

6. Verwendung nach einem der Ansprüche 1-5, bei der die Farbentwicklerlösung, die zur Entwicklung des Materials verwendet wird, auch ein Pyrazolidinon der Formeln (I) oder (II), wie in Anspruch 1 definiert, enthält.

7. Verwendung nach Anspruch 6, bei der die Farbentwicklerlösung 0,05 bis 5,0 g/l des Pyrazolidinons enthält.

8. Verwendung nach Anspruch 6, bei der die Farbentwicklerlösung 0,1 bis 1,0 g/l des Pyrazolidinons enthält.

9. Verwendung nach einem der Ansprüche 1-8, bei der das Farb-Negativmaterial ein mehrfarbiges photographisches Material ist mit einem Träger, auf dem sich befinden eine ein gelbes Farbstoffbild bildende Einheit mit mindestens einer blau-empfindlichen Silberhalogenidemulsionsschicht, der mindestens ein einen gelben Farbstoff bildender Kuppler zugeordnet ist, mindestens eine ein purpurrotes Farbstoffbild liefernde Einheit mit mindestens einer grün-empfindlichen Silberhalogenidemulsionsschicht, der mindestens ein einen purpurroten Farbstoff liefernder Kuppler zugeordnet ist, und mindestens eine ein blaugrünes Farbstoffbild liefernde Einheit mit mindestens einer rot-empfindlichen Silberhalogenidemulsionsschicht, der mindestens ein einen blaugrünen Farbstoff liefernder Kuppler zugeordnet ist.

10. Verwendung nach einem der Ansprüche 1-9, bei der das Pyrazolidinon in oder benachbart zur Silberhalogenidemulsionsschicht, die dem Träger am nächsten liegt, angeordnet ist.

## Revendications

1. Utilisation d'un composé pyrazolidinone de formule : or ou d'un précurseur de celui-ci libérant le composé pyrazolidinone au cours du traitement avec une solution de traitement alcaline, afin de réduire la granularité d'un produit photographique négatif en couleurs aux halogénures d'argent traité et exposé en conformité avec une image, comprenant un support portant au moins une couche d'émulsion aux halogénures d'argent photosensible à laquelle est associé un coupleur formateur de colorant d'image et contenant une quantité de composé pyrazolidinone telle que l'on réduit la granularité sans modifier la densité du colorant pour un même niveau d'exposition.

2. Utilisation selon la revendication 1, dans lequel le précurseur est un composé ballasté qui libère le composé pyrazolidinone lorsqu'il est mis en contact avec une solution de développement chromogène alcaline.

3. Utilisation selon la revendication 2, dans lequel le précurseur pyrazolidinone est représenté par l'une des formules : ou où R¹ et R² sont des groupes alkyle ou aryle pouvant être substitués et où R¹ et R² ont une taille et une configuration telles qu'ils ne permettent pas au précurseur de migrer dans les couches photographiques.

4. Utilisation selon l'une quelconque des revendications 1 à 3, dans lequel le produit négatif en couleurs est un film contenant de 0,01 à 5,0 g/m² de composé pyrazolidinone.

5. Utilisation selon l'une quelconque des revendications 1 à 3, dans lequel le produit négatif en couleurs est un film contenant de 0,05 à 1,0 g/m² de composé pyrazolidinone.

6. Utilisation selon l'une quelconque des revendications 1 à 5, dans lequel la solution de développement chromogène utilisée pour traiter le produit contient également un composé pyrazolidinone de formule (I) ou (II), tel que défini dans la revendication 1.

7. Utilisation selon la revendication 6, dans lequel la solution de développement chromogène contient de 0,05 à 5,0 g/l de composé pyrazolidinone.

8. Utilisation selon la revendication 6, dans lequel la solution de développement chromogène contient de 0,1 à 1,0 g/l de composé pyrazolidinone.

9. Utilisation selon l'une quelconque des revendications 1-8, dans lequel le produit négatif en couleurs est un produit photographique multicolore comprenant un support portant une unité formatrice d'image de colorant jaune constituée d'au moins une couche d'émulsion aux halogénures d'argent sensible au bleu à laquelle est associé au moins un coupleur formateur de colorant d'image jaune, au moins une unité formatrice d'image de colorant magenta constituée d'au moins une couche d'émulsion aux halogénures d'argent sensible au vert à laquelle est associé au moins un coupleur formateur de colorant d'image magenta et au moins une unité formatrice d'image de colorant cyan constituée d'au moins une couche d'émulsion aux halogénures d'argent sensible au rouge à laquelle est associé au moins un coupleur formateur de colorant d'image cyan.

10. Utilisation selon l'une quelconque des revendications 1-9, dans lequel le composé pyrazolidinone est placé dans la couche d'émulsion aux halogénures d'argent la plus proche du support ou dans une couche adjacente.
